

March 24, 1964

M. BAEBLER

3,125,848

YARN AND FABRIC PRODUCT AND PROCESS

Original Filed Nov. 7, 1956



INVENTOR.  
MARIJAN BAEBLER

BY  
Ward, Neal, Haseltine  
Orme & McElhenny  
his ATTORNEYS.

1

3,125,848

**YARN AND FABRIC PRODUCT AND PROCESS**  
Marijan Baebler, Wattwil, Switzerland, assignor to Heberlein Patent Corporation, New York, N.Y., a corporation of New York  
Continuation of applications Ser. Nos. 620,957 and 620,958, Nov. 7, 1956. This application Dec. 27, 1962, Ser. No. 248,841  
24 Claims. (Cl. 57—140)

This invention relates to a process for making an improved stretch nylon or similar organic synthetic fiber yarn, and to the yarn product. It also relates to articles, including hosiery, made from the improved stretch yarn and to a process for making such articles. This application is a continuation of both of my earlier copending United States patent applications Serial Numbers 620,957 and 620,958 both filed November 7, 1956, and both now abandoned.

In Billion U.S. Patent 2,564,245 a process is described for producing superpolyamidic yarn having permanent crimping and fluffing properties. The superpolyamidic yarn is highly twisted, set and backtwisted, during which process it shrinks. The yarn is plied with another yarn treated in the same manner but twisted in an opposite way. The yarns so plied, having respectively an S-twist and a Z-twist, thus compensate one another, so that the resultant yarn has practically no directional torque. This is the conventional process which has been widely practiced commercially. Socks and stockings made of stretch nylon prepared in accordance with the Billion patent are well known. Such hosiery is ordinarily made of plied stretch yarn as aforesaid, or it may also be fabricated of S and Z yarns knitted or woven to give a compensated effect.

Where S and Z yarns are plied, each yarn must be individually processed under about the same conditions except for the direction of twist, in order to produce a compensated yarn. In addition, with such composite yarn it must be made of at least two yarns, each having one-half of the denier desired in the finished yarn.

An object of the present invention is to provide a process for producing a single end yarn which does not require the plying together for compensation of two yarns, each with an opposite directional torque; and to produce thereby a product ready for knitting or other use.

Another object of the present invention is to provide a woven or knitted article such as a sock or stocking made of yarn which does not require such compensation of torque therein.

In carrying out my process for producing yarn I employ a yarn of synthetic organic fiber, by which expression I intend to define polyamidic fibers, such as those made from polyhexamethylene adipamide or from epsilon-caprolactam, polyacrylonitrilic fibers and polyester fibers. The yarn employed usually comes on the market with relative few turns per meter, namely about 0 to 80 turns per meter. Such yarn, in highly twisted state, is originally set in the first step by heating in accordance with my invention. By "highly twisted" in this first step I mean a yarn that is twisted at a twist of the order of about 1000 to 6000 turns per meter. This yarn is set originally at a temperature of the order of 100 to 225° C. I prefer to carry out this twisting and setting by the so-called false-twisting process, which is a well known process by which the yarn is continuously passed through a heating zone and is set therein while being continuously highly twisted to the extent indicated, and detwisted. The temperature and high-twist ranges above are used where false-twisting is employed. Instead of the false twisting mentioned, the conventional steps referred to above may be employed

2

in this original setting and detwisting. In the second step the yarn so set and detwisted by the false-twist or conventional process is then retwisted to no higher number of twists than in the first step, in the opposite direction, and is reset in this condition. The retwisting and resetting again are preferably done in a false twisting machine. The number of twists placed in yarn in both false twist and conventional methods may be equal or different in the second step from the number of twists in the first step. The resetting temperature range for false twists is 100–225° C. For the conventional method, the resetting is done with saturated steam at 0–5 atm. gauge pressure. Either or both steps 1 and 2 may be made accordingly by the false twist or conventional method.

15 In carrying out my process, the retwisting is thus done at the same or a lower number of twists and the resetting at the same or a lower temperature than in the original or first setting step. After retwisting and resetting detwisting occurs. In the false twisting method the detwisting is substantially to the number of twists of the gray yarn. In the conventional process the detwisting may be to zero or several twists in the S or Z direction with respect to zero.

20 Yarn so produced is permanently crimped and has good inherent elasticity. It is a single end multi-filament yarn. The yarn has a torque or twist which develops on wetting as described below. Thus the yarn resulting from the two steps of my process may show no actual torque, but on wetting a torque will develop. This torque will

25 be in the direction, either S or Z, of the twist given the yarn in the first step. On the other hand, yarn produced from the two steps of my process may show an actual torque and this actual torque will be in the direction of the twist given the yarn by the second step of my process, namely, in either Z or S direction. In such case,

30 when this yarn is wetted as described below, it will develop a torque due to and in the direction of the twist in the first step. If this torque or twist of the first step so developed by wetting equals the actual torque of the second step, then the yarn will become a yarn without substantial torque. If the torque developed on wetting is greater than the actual torque of the second step, then the final yarn on wetting will have a torque in the direction of the first step. If it is less than the torque of the second step, then the resultant yarn will have the torque of the second step.

35 My novel fabric product includes a woven or knitted article containing a permanent elastic crimp single-end yarn of organic synthetic fibers as above described. The 40 yarn has a torque S or Z, which develops on wetting the yarn, as noted above. Ordinarily, it also has an actual torque which is substantially equal to and in the opposite direction to the torque which develops on wetting, that is the "wet" torque.

45 45 The wetting treatment referred to above defines treatments to which yarns are normally subjected in scouring, dyeing or boarding knit or woven fabrics. An important characteristic of my improved yarn is that on knitting a fabric produced from a yarn having an actual torque,

50 50 the resulting fabric will have wales inclined to the vertical in the opposite direction to that of the torque. For example, a yarn with an S torque will produce a fabric with wales inclined in a Z direction and vice versa. On wetting such fabric, the wales will change to a substantially vertical position if the torque developed on wetting is equal to the actual torque of the yarn. If it is unequal, the wales will incline either in the same direction as the wet torque or in the opposite direction to the wet torque,

55 55 depending on whether the torque is greater or less than the actual torque.

60 60 In accordance with one aspect of the present invention I may knit a yarn in which the wet torque has been de-

veloped by scouring or dyeing, for example, into an article after this finishing treatment, and if its actual and wet torques are equal such knitting will produce a fabric with vertical wales.

In the accompanying drawings forming part of this application:

FIG. 1 shows a doubled length of stretch nylon yarn freely suspended, made in accordance with my invention for making yarn.

FIG. 2 is a microscopic, highly enlarged portion of the yarn shown in FIG. 1, said portion being designated by a bracket in FIG. 1, and marked "FIG. 2."

FIG. 3 is a portion of a knitted fabric which has an angular distortion in the  $\mathfrak{S}$  direction.

FIG. 4 is a highly enlarged and schematic view of the fabric shown in FIG. 3.

FIG. 5 is the fabric of FIG. 3 after wetting same, showing the wales in vertical position.

FIG. 6 is a highly enlarged and schematic view of the fabric shown in FIG. 5, with the wales in vertical position.

For simplicity the yarns in FIGS. 3-6 are shown in smooth form. They would actually appear somewhat fuzzy as in FIG. 1.

Referring now to the figures, the numeral 1 designates a strand of the nylon yarn which has been doubled and then freely suspended. The yarn has an actual unidirectional torque and accordingly tends to turn about the vertical axis, forming a series of wide loops marked 2. The amount of torque is small, as shown by the relatively few large loops formed.

In FIG. 2 the microscopic enlargement of the portion of the strand 1 shows that this strand is made up of filaments which are crimped and irregularly intertwined with one another in a form characteristic of stretch nylon yarn.

The strand 1, as stated, has an actual unidirectional torque or tendency to twist about its vertical axis when held in the form of a doubled loop. This yarn has a wet torque, that is, a torque which is developed by wetting same as described above. If this yarn has a wetting torque equal to the actual torque, the resulting yarn on wetting will be a yarn without torque. On the other hand, as stated above, if the wet torque is greater than the actual torque then the yarn will have a torque in the direction of the wet torque. If it is less than the actual torque then the yarn on wetting will have a torque in the direction of the actual torque.

Referring to FIG. 3, the knitted fabric there shown has wales inclined to the vertical in the  $\mathfrak{S}$  direction. When the yarn shown in FIG. 1 is knit into fabric as shown in FIG. 3, this inclination occurs because of the unidirectional actual torque of the yarn. In the highly enlarged showing in FIG. 4 the wales 3 are shown as extending from left to right at a small angle with respect to the vertical axis of the fabric. The yarn also has a wet torque which is substantially equal to the actual torque. On wetting the fabric, as above stated, the wet torque appears and the wales become vertical. Wetting may be done by simple immersion of the fabric in water or by ordinary finishing processes as above stated at times and temperatures depending on the conditions of treatment of the yarn, and the character of the yarn, in accordance with my invention.

Thus in FIG. 5 is shown the fabric of FIG. 3 after such wetting treatment. It will be noted that the wales 3 are substantially vertical. In other words, the inclination shown in FIGS. 3 and 4 has been corrected so that the wales are in the vertical position as shown in FIGS. 5 and 6.

In using nylon yarn, if the conditions of temperature and twist for the first and second steps are not carefully observed, the wales may not appear in exactly vertical position on wetting. In other words, they may have an angle of inclination to the vertical. For some fabrics this is not objectionable, but for the majority of fabrics,

including socks and stockings, it is important that the wales be vertical.

Instead of knitting the sock or other fabric and then correcting the angular distortion by wetting, the yarn itself employed in the fabric may be wet to produce a yarn without substantial torque, and such yarn may then be employed for knitting purposes to give a fabric with substantially vertical wales.

The following are examples of the manner in which I now prefer to practice my invention. It is to be understood that the examples are illustrative, and the invention is not intended to be limited thereto, except as indicated in the appended claims.

#### EXAMPLE 1

First step: A polyamide yarn, made of the polycondensation-product of hexamethylenediamine and adipic acid, 7 den., 23 filaments with a twist of 30 t./m.  $Z$  is hightwisted on a ring-twisting machine to approximately 3000 t./m.  $Z$ , set during 20 minutes with saturated steam at 2 atm. gauge pressure and then detwisted beyond the zero point to approximately 200 t./m.  $S$ . Second step: Then the yarn is temporarily hightwisted on a falsetwisting machine to approximately 2000 t./m.  $S$  and in this highly twisted state steamed at 1.5 atm. gauge pressure for approximately 1.5 seconds. One obtains therewith a permanent intensely and evenly crimped inherently elastic single yarn. The yarn so produced has a crimp retentivity of 73% and a maximum elongation of 210%.

#### EXAMPLE 2

First step: A polyamide yarn, made of the polycondensation-product of hexamethylene diamine and adipic acid (nylon) 30 den., 10 filaments with a twist of 30 t./m.  $Z$  is temporarily hightwisted by means of a falsetwisting machine to approximately 4500 t./m.  $S$  and in this hightwisted state set with saturated steam at 4.5 atm. gauge pressure for 2 seconds. Then, in a second step, the yarn is hightwisted with a falsetwisting machine to approximately 4500 t./m.  $Z$ , whereby it is set with saturated steam in the hightwisted state at 1 atm. gauge pressure for 2 seconds. One obtains by this procedure a permanent single inherently elastic crimped yarn, with a pleasant hand. The yarn so produced has a crimp retentivity of 87% and a maximum elongation of 150%.

#### EXAMPLE 3

First step: A polyamide yarn, as mentioned in Example 1, is hightwisted on a ringtwisting machine to approximately 3000 t./m.  $Z$ , set with saturated steam at 2 atm. gauge pressure during 20 minutes and detwisted beyond the zero point to approximately 56 t./m.  $S$ . Second step: Then, the yarn is hightwisted on a falsetwisting machine to approximately 3000 t./m.  $S$  and fixed in this hightwisted state with hot air of 180° C. during 1.5 seconds. One obtains therewith, an inherently elastic single, crimped yarn. The yarn so produced has a crimp retentivity of 76% and a maximum elongation of 190%.

#### EXAMPLE 4

First step: A nylon yarn 30 den., 10 filaments with a twist of 280 t./m.  $Z$  is temporarily hightwisted by means of a falsetwisting machine to approximately 4500 t./m.  $S$  and set in the hightwisted state with hot air of 225° C. during 1.9 seconds. Then in the second step, the yarn is hightwisted on a falsetwisting machine to approximately 3000 t./m.  $Z$ , whereby it is heated in the hightwisted state with hot air of 175-180° C. during approximately 1.6 seconds. The single crimped yarn produced is inherently highly elastic. The yarn so produced has a crimp retentivity of 89% and a maximum elongation of 110%.

#### EXAMPLE 5

First step: A polyamide yarn, as per Example 1, is hightwisted on a ringtwisting machine to approximately 3000 75 t./m.  $Z$ , set with saturated steam at 2 atm. pressure dur-

ing 20 minutes and detwisted beyond the zero point to approximately 230 t./m. **S**. Second step: Then the yarn is hightwisted on a ringtwisting machine to approximately 2000 t./m. **S** and set with saturated steam at 0.3 atm. gauge pressure during 5 minutes, and then detwisted beyond the zero point to approximately 110 t./m. **Z**. One obtains inherently, highly elastic, crimped yarn with a pleasant hand. The yarn so produced has a crimp retentivity of 70% and a maximum elongation of 210%.

## EXAMPLE 6

First step: A nylon yarn 30 den., 10 filaments, with a twist of 30 t./m. **Z** is temporarily hightwisted by means of a falsetwisting machine to approximately 4500 t./m. **S** and set in the hightwisted state at a temperature of 200° C. during 3 seconds by means of an electrical heating unit, as described in the United States patent application Serial No. 601,202, now U.S. Patent No. 2,823,292. Then in the second step the yarn is hightwisted on a falsetwisting machine to approximately 3500 t./m. **Z**, whereby it is heated in the hightwisted state with hot air of 160° C. during 2.2 seconds. The yarn so produced has a crimp retentivity of 89% and a maximum elongation of 160%.

## EXAMPLE 7

First step: A nylon yarn 30 den., 10 filaments, with a

means of a falsetwisting machine to approximately 4000 t./m. **Z** and set in the hightwisted state with hot air of 220° C. during 2.4 seconds. Second step: Thereupon, the yarn is temporarily hightwisted with a falsetwisting machine to approximately 2650 t./m. **S** and set in the hightwisted state with hot air of 150° C. during 1.8 seconds. The highly elastic crimped yarn produced has a twist of approximately 160 t./m. **S**, a crimp retentivity of 87%, and a maximum elongation of 140%.

10

15

20

EXAMPLE 11

First step: A polyester yarn of polyethyleneglycol-terephthalate 100 den., 48 filaments, with a twist of 30 t./m. **S** is hightwisted on a ringtwisting machine to approximately 2400 t./m. **S** and set in the hightwisted state with saturated steam of 3 atm. gauge pressure during 20 minutes. Then the yarn is detwisted on the ringtwisting machine beyond the zero point to about 120 t./m. **Z**. Second step: Thereupon the so treated yarn is temporarily hightwisted by means of a falsetwisting machine to approximately 1600 t./m. **Z** and set in the hightwisted state with hot air of 140° C. during 1 second. There is obtained a highly elastic crimped yarn with a twist of 120 t./m. **Z** having a crimp retentivity of 82%.

The following is a tabulation of additional tests carried out on nylon yarn:

|                 | Denier | Hot Air Temp., ° C. <sup>2</sup> | Twist <sup>1</sup>            | Hot Air Temp., ° C. <sup>2</sup> | Approx. Time (Secs.) |        | Twist <sup>2</sup>            | Crimp Retentivity, Percent | Maximum Elonga-tion, Percent |
|-----------------|--------|----------------------------------|-------------------------------|----------------------------------|----------------------|--------|-------------------------------|----------------------------|------------------------------|
|                 |        |                                  |                               |                                  | Step 1               | Step 2 |                               |                            |                              |
| Example 12----- | 15/3   | 220                              | 4,724.40 t./m. <b>Z</b> ----- | 161                              | 2.5                  | 1.5    | 2,952.75 t./m. <b>S</b> ----- | 94                         | 213                          |
| Example 13----- | 30/10  | 220                              | 4,429.13 t./m. <b>Z</b> ----- | 170                              | 2                    | 1.5    | 2,952.75 t./m. <b>S</b> ----- | 89                         | 131                          |
| Example 14----- | 70/34  | 220                              | 3,110.23 t./m. <b>Z</b> ----- | 170                              | 1.5                  | 1.2    | 2,362.20 t./m. <b>S</b> ----- | 70                         | 100                          |
| Example 15----- | 140/68 | 220                              | 2,362.20 t./m. <b>S</b> ----- | 172                              | 1.5                  | 1.1    | 1,748.03 t./m. <b>Z</b> ----- | 70                         | 63                           |

<sup>1</sup> First step.

<sup>2</sup> Second step.

twist of 30 t./m. **Z** is temporarily hightwisted and set in the hightwisted state under conditions as described in Example 6. Then in a second step the yarn is hightwisted in a falsetwisting machine to about 300 t./m. **Z** and heated in the hightwisted state at a temperature of 170° C. during 1.9 seconds by means of an electrical heating unit. The yarn so produced has a crimp retentivity of 95% and a maximum elongation of 150%.

## EXAMPLE 8

First step: A nylon yarn, 20 den., 7 filaments, with a twist of 16 t./m. **Z** is temporarily hightwisted on a falsetwisting machine to approximately 5000 t./m. **Z** and set in the hightwisted state during 3.1 seconds at a temperature of 225° C. by means of an electrical heating unit, as described in the aforementioned United States patent application Serial No. 601,202<sup>1</sup>. Then in a second step the yarn is falsetwisted to about 4000 t./m. **S** and heated in the hightwisted state with hot air of 170° C. during 2.5 seconds. The yarn so produced has a crimp retentivity of 88% and a maximum elongation of 180%.

## EXAMPLE 9

First step: A nylon yarn, 20 den., 7 filaments, with a twist of 16 t./m. **Z** is falsetwisted and set in the hightwisted state under conditions as described in Example 8. Then in a second step the yarn is falsetwisted to about 3500 t./m. **S** and heated in the hightwisted state with hot air of 180° C. during 2.2 seconds. The yarn so produced has a crimp retentivity of 90% and a maximum elongation of 200%.

## EXAMPLE 10

First step: A polyester yarn of polyethyleneglycol-terephthalate 40 den., 24 filaments, with a twist of 30 t./m. **S** is twisted on a ringtwisting machine to approximately 160 t./m. **S**. Then the yarn is temporarily hightwisted by

In each of Examples 1 to 15, the tension of the yarn will vary between 0-15 grams depending on the denier; the lower the denier, the less tension is required.

Yarns made by Examples 1 to 15 upon completion of step 1 are shrunk yarns, i.e., yarns without residual shrinkage. Step 2 is conducted on such shrunk yarn and, so far as I am aware, no such twisting, setting and detwisting of shrunk yarn has heretofore been proposed.

In order to measure crimp retentivity and maximum elongation of a yarn treated according to my process, the yarn must primarily be allowed to crimp completely. This is performed by exposing the yarn in the form of a small skein for about 5 minutes to the action of moist steam thereby allowing the yarn to contract freely. Sized or oiled yarn should be washed free of extraneous substances before steaming. The crimped yarn is then conditioned at 20° centigrade and 65 percent relative humidity.

To determine crimp retentivity, a length of 30 centimeters of the completely crimped yarn is suspended on one end and after preloading for 2 minutes with 0.002 g. per denier the exact length (*a*) of the preloaded yarn is measured. The yarn is then immersed for 30 seconds in water of 60° centigrade containing 2 g. of wetting agent of the type of "Nekal BX" (General Dyestuff Corp.); thereafter the wet yarn is suspended for two minutes with a load of 0.03 g. per denier and the length (*b*) of the stretched yarn measured. After taking off the load, the yarn is dried without any tension at 50° to 60° centigrade. After being conditioned for one hour at 20° centigrade and 65 percent relative humidity, the yarn is loaded for two minutes with 0.002 g. per denier and its length (*c*) measured. The crimp retentivity in percent is then calculated according to the following formula:

$$\frac{b-c}{b-a} \cdot 100$$

To determine maximum elongation a length of about

<sup>1</sup> Now Patent No. 2,823,292.

30 centimeters of the completely crimped yarn is suspended on one end and preloaded with 0.002 g. per denier for 2 minutes, whereupon the exact length ( $x$ ) of the preloaded yarn is measured. The yarn is now loaded with 0.8 g. per denier for two minutes and then the length ( $y$ ) of the so stretched yarn is measured. The maximum elongation in percent is calculated according to the formula below:

$$\frac{y-x}{x} \cdot 100$$

10

The yarn of each of the above examples is then formed into a stocking as for instance in the manner described in Example 16 below. The stocking is then scoured in a relaxed condition at 60-70° C. for 30 minutes in a bath containing 2 grams "Igepal" CO-630 (or equivalent non-ionic washing agent) and 0.5 gr. soda ash per liter of water, rinsed for 3 minutes with warm (about 50° C.) water and then 5 minutes in cold tap water, then carefully centrifuged and dried in a relaxed condition at about 50° C.

Prior to the scouring operation mentioned the knitted material will show wales inclined to the vertical. The direction of the inclination will be in the direction opposite to that of the second high twisting operation. Upon scouring the knitted material as above, however, this inclination is substantially eliminated and the knitted material thereafter shows vertical wales. The scouring thus not only cleans the goods, but also removes the inclination, as indicated above.

The following are further specific examples of the manufacture of hosiery in accordance with my invention. Yarn in accordance with my invention is prepared, then carried through specific processes of hosiery knitting, both circular and full-fashioned knitting, followed by 35 specific dyeing and other finishing steps.

#### EXAMPLE 16.—STOCKING FROM 15-DENIER YARN

The yarn was prepared in accordance with the procedure in Example 12 above.

##### Knitting

Knit on Scott & Williams circular knitting machine 400 needles, 3 1/4" cylinder under "drag tension," that is, the tension exerted on the yarn by the knitting machine but without any tension applied such as by a spring or disc tension. The needles are .75 gauge and the latches 80 gauge. Heel and toe and welt are made of normal yarn in the usual manner. Knit under normal conditions.

The stocking has wales inclined to the vertical.

##### Dyeing and Finishing

(1) The stocking is scoured in a bath containing a mild soap for 20-30 minutes at a temperature not to exceed 65° C.

(2) The stocking is then dyed with dispersion dyestuffs for 20-30 minutes in a bath whose temperature is about 65° C.

(3) The boarding is carried out on a small form for 2 minutes at a steam temperature of 116° C.

The above steps of dyeing and finishing are the same as used for other stretch stockings, that is, they constitute standard practice.

The stocking so produced shows a dull mat effect. Its wales are substantially vertical. It has substantially no shine. It has a good hand, that is, it is softer than stockings knit from untreated nylon. It has a better fit than such stockings due to its stretch character.

#### EXAMPLE 17.—SOCK FROM 140-DENIER POLY-AMIDE YARN

The yarn employed herein was prepared in accordance with Example 15 above. The yarn was knit on a Scott & Williams circular knitting machine as above in Example 16 with respective needle spacing. The socks so

knitted were put in a bag and washed in water at a temperature of 50° to 65° C. for 15-20 minutes. The socks then showed vertical wales. They were then preboarded at 116° C. for 1 1/2 minutes at dry heat. They were then dyed at about 65° C. using neutral dyeing acid dyestuffs. They were then finished in the usual manner.

The socks showed a dull mat appearance. They are better fitting, due to their stretch character, than socks knit from ordinary 140-denier nylon. They have a good soft hand.

The dyeing in each of Examples 16 and 17 was made with dyestuffs selected from the following: DuPont acetamide yellow N; DuPont acetamide yellow CG (Pr 242); DuPont acetamide scarlet N; and DuPont acetamide blue FS. The temperature of the dye baths may range from 60° C.-70° C.

#### EXAMPLE 18.—STOCKING MADE FROM 40-DENIER POLYESTER YARN

##### Knitting

The yarn employed herein was prepared in accordance with Example 10 above. The yarn was knit on a Scott & Williams circular knitting machine 300 needles, 3 1/2" cylinder under slight tension.

##### Dyeing and Finishing

The stocking was scoured in a bath containing 2 grams "Igepal" CO 630 (which is a polymerized ethylene oxide-alkyl phenol condensation product) and 0.5 gram soda ash per liter of water for 30 minutes at 60° C., rinsed first with warm and then with cold water. The dyeing was performed in a bath containing per liter 1 gram of the sodium salt of the oleyl-alcohol-sulphate and the following dyestuffs:

|                                               | Percent |
|-----------------------------------------------|---------|
| "Celanthrene" Fast Yellow conc. 300% (Pr 534) | 1.03    |
| "Acetamine" Orange GR conc. 175% (Pr 43)      | 0.04    |
| "Celanthrene" Brill. Blue FR conc. (Pr 228)   | 0.01    |

<sup>1</sup>Percent based on the dry weight of the goods to be dyed.

The stocking was entered into the dyebath at 50° C., whereupon the temperature of the liquor was slowly raised to the boil and maintained at that temperature for one hour. Finally the stocking was boarded on a small form at a steam temperature of 110° C.

The stocking so produced shows a reduced lustre, a soft silky hand and has a good fit due to stretch character.

I claim:

1. A method of making a continuous filament stretch yarn of the synthetic resinous type which comprises subjecting the yarn to a first false twist in one direction and heat setting the yarn and subsequently subjecting the so twisted and heat-set yarn to a false twist in the opposite direction and heat treating in the second stage of false twist at a temperature lower than in the first stage.

2. A method as set forth in claim 1 wherein the false twist in the second stage is to a lower number of twists than the first false twist.

3. A method as set forth in claim 1 wherein the false twist in the second stage is to substantially the same number of twists as the first false twist.

4. A method of making a stable stretch multifilament yarn of the synthetic resinous type which comprises subjecting the yarn to a first false twist of at least 30 twists per linear inch in one direction and heat setting the yarn and subsequently subjecting the so twisted and heat-set yarn to substantially the same degree of false twist but in the opposite direction and heat-treating the yarn in the second stage of false twist at a temperature lower than in the first stage.

5. A method of making a continuous filament stretch yarn of the synthetic resinous type which comprises subjecting the yarn to a first false twist in one direction and heat setting the yarn and subsequently subjecting the so twisted and heat-set yarn to a false twist in the opposite

direction and heat treating in the second stage of false twist at a temperature substantially the same as in the first stage.

6. A method of making a continuous filament stretch yarn of the synthetic resinous type which comprises subjecting the yarn in a first stage to a false twist in one direction and heat-setting the yarn whereby a torque is imparted to the so treated yarn in a direction opposite to the direction of twist and subsequently subjecting the so twisted and heat-set yarn in a second stage to a false twist in the direction opposite to that of the first stage false twist, and heat-treating the entire yarn in the second stage of false twist, the false twist and temperature to which the yarn is heated in the second stage being no greater than in the first stage.

7. A method of making a continuous filament stretch yarn of the synthetic resinous type which comprises subjecting the yarn to a first false twist of the order of about 1000 to 6000 turns per meter and heat setting the yarn and subsequently subjecting the so twisted and heat-set yarn to a false twist in the opposite direction and heat treating the entire yarn in the second stage of false twist at a temperature of the order of about 100 to 225° C., but no higher than in the first stage false twist.

8. A process as set forth in claim 7 wherein heat treating in the second stage of false twist is at a temperature lower than in the first stage.

9. A process as set forth in claim 7 wherein heat setting of the yarn in the first stage of false twist is at a temperature of the order of about 160 to 225° C.

10. A process as set forth in claim 7 wherein the false twist in the opposite direction is of the order of about 400 to 6000 turns per meter.

11. A continuous method for producing a continuous filament stretch yarn of the synthetic resinous type which comprises continuously subjecting a raw continuous filament synthetic resinous yarn in a first stage to a false twist in one direction and heat-setting the yarn whereby a torque is imparted to the so treated yarn in a direction opposite to the direction of twist, and immediately thereafter continuously subjecting the so twisted and heat-set yarn in a second stage to a false twist in the direction opposite to that of the first stage false twist, and heat-treating the entire yarn in the second stage of false twist, the false twist and the temperature to which the yarn is heated in the second stage being no greater than in the first stage.

12. A false twisted substantially uniform permanently crimped continuous filament stretchable single-end yarn of the synthetic resinous type having an actual unidirectional torque and a latent torque which develops on wetting and is in the opposite direction to said actual torque.

13. A multifilament nylon yarn as set forth in claim 12.

14. A false twisted permanently crimped continuous

filament stretchable single-end yarn of the synthetic resinous type having an actual unidirectional torque and an opposite latent torque which develops on wetting and is less than the actual torque of the yarn.

5 15. A false twisted permanently crimped continuous filament stretchable single-end yarn of the synthetic resinous type having an actual unidirectional torque and an opposite latent torque which develops on wetting and is greater than the actual torque of the yarn.

10 16. A false twisted permanently crimped continuous filament stretchable single-end yarn of the synthetic resinous type having an actual unidirectional torque and an opposite latent torque which develops on wetting and is substantially equal to the actual torque of the yarn.

15 17. A permanently crimped continuous multifilament stretchable single-end yarn of the synthetic resinous type false twisted and heat set over its entire length which exhibits substantially no torque following wetting.

18. A permanently crimped continuous filament stretchable single-end yarn of the synthetic resinous type false twisted and heat set over its entire length which exhibits substantially no torque prior to wetting but exhibits torque following wetting.

25 19. A fabric fashioned of a permanently crimped, highly stretchable, single-end, multifilament synthetic organic yarn, which fabric exhibits a tendency to curl prior to wetting but substantially no tendency to curl following wetting.

30 20. A fabric fashioned of a single-end of permanently crimped, highly stretchable, multifilament synthetic organic yarn, which yarn exhibits torque prior to wetting but substantially no torque following wetting.

35 21. A fabric fashioned of permanently crimped, highly stretchable, single-end multifilament synthetic organic yarn, the filaments of which are irregularly intertwined, all of which yarn exhibits a unidirectional torque prior to wetting and substantially no torque following wetting.

40 22. A knit fabric fashioned of a single-end of permanently crimped, highly stretchable, multifilament synthetic organic yarn, which yarn exhibits torque prior to wetting but substantially no torque following wetting.

45 23. A knit fabric having a tendency to curl following wetting as evidenced by inclination of the wales thereof from the vertical fashioned of the single-end yarn of claim 15.

24. A method as set forth in claim 1 wherein the continuous filament stretch yarn is a multifilament yarn.

#### References Cited in the file of this patent

#### UNITED STATES PATENTS

|           |                       |                |
|-----------|-----------------------|----------------|
| 2,353,666 | Hathorne et al. ----- | July 18, 1944  |
| 2,755,616 | Weller -----          | July 24, 1956  |
| 2,807,073 | Stuewer -----         | Sept. 24, 1957 |
| 2,909,028 | Comer et al. -----    | Oct. 20, 1959  |

UNITED STATES PATENT OFFICE  
CERTIFICATE OF CORRECTION

Patent No. 3,125,848

March 24, 1964

Marijan Baebler

It is hereby certified that error appears in the above numbered patent requiring correction and that the said Letters Patent should read as corrected below.

Column 4, line 17, for "7 den." read -- 70 den. --; column 5, line 41, for "300 t./m." read -- 3000 t./m. --.

Signed and sealed this 4th day of August 1964.

(SEAL)

Attest:

ERNEST W. SWIDER  
Attesting Officer

EDWARD J. BRENNER  
Commissioner of Patents